

## UNITED STATES PATENT OFFICE

2,231,010

## HEAT TREATING PROCESS

Donald A. Holt, Niagara Falls, N. Y., assignor to  
E. I. du Pont de Nemours & Company, Wil-  
mington, Del., a corporation of Delaware

No Drawing. Original application February 24,  
1938, Serial No. 192,396. Divided and this ap-  
plication May 20, 1940, Serial No. 336,178

4 Claims. (Cl. 148—15)

This invention relates to the heat treatment of metal articles and more particularly to heat treatment by means of fused salt baths.

This application is a division of my copending 5 patent application Serial No. 192,396, filed February 24, 1938.

Heat treating operations for articles of various metals are often carried out by immersing the metal articles to be treated in a fused salt bath.

10 This method of heat treatment is advantageous because of the rapid transfer of heat from the bath to the metal articles, thus providing a rapid process well adapted to large scale production. Heat treating fused salt baths which contain 15 no carburizing agent, for example alkali metal cyanide or other cyanogen compound, are known to have a more or less decarburizing effect upon steel surfaces, which effect has been overcome heretofore by introducing a carburizing mate- 20 rial into the bath. By this method the carburization which occurs more or less compensates for the decarburizing effect of the bath. This method of controlling the carburizing activity of baths containing a cyanogen compound is not 25 particularly reliable or satisfactory. Moreover, it is often desired to employ baths which will exert a substantial and controllable carburizing action upon steel articles immersed therein. So far as I am aware, there has been no really satis- 30 factory method available for practically controlling the carburizing activity of fused salt baths which contain a cyanogen compound.

It is an object of the present invention to provide a new and improved method for controlling the activity of fused salt case hardening 35 baths which contain a carburizing material. A further object is to provide a method of operating fused salt baths containing a cyanogen compound whereby the case hardening activity of the bath may be inhibited or controlled as 40 desired. Still further objects will be apparent from the ensuing description of the invention.

The above objects are accomplished in accordance with my invention by heating metal articles in a fused salt bath containing a cyanogen compound, while maintaining said bath in an atmosphere of a gas containing a predetermined amount of an oxidizing constituent. I have discovered that a fused salt bath which contains a 45 cyanogen compound, such as sodium cyanide, may be rendered substantially inert as regards carburizing or decarburizing activity, by maintaining the bath in an atmosphere of an oxy- 50 gen-free, non-oxidizing gas, as described and claimed in my copending application Serial No. 192,396, filed February 24, 1938. I have also discovered that the case hardening activity of such a bath increases as the amount of oxidizing 55 constituent in the gaseous atmosphere main- 60

tained over the bath is increased, and that by varying the amount of oxidizing constituent in the gaseous atmosphere, the case hardening activity of the bath may be varied accordingly.

The fused case hardening baths to be used 5 in practicing the present invention of course must contain a carburizing material such as an alkali metal cyanide. Alkaline earth metal cyanides and cyanamides, as well as other cyanogen compounds, such as polymers of hydrocyanic acid, 10 cyanamide, dicyandiamide and its polymers, may be used as carburizing bath ingredients. The amount of carburizing material present in the bath may be varied over a wide range. Thus, the bath may contain 0.5 to 40% by weight of 15 sodium cyanide, or if desired, a bath of substantially pure sodium cyanide may be employed with good results.

The case hardening baths for use in practicing my invention preferably contain as the chief 20 bath constituents a cyanogen compound and an alkali metal salt, an alkaline earth metal salt, or mixtures thereof. In particular, I prefer to use baths containing sodium cyanide together with alkali metal and alkaline earth metal hal- 25 ides and carbonates, or mixtures thereof. The methods of mixing and fusing the salt ingredients of the bath, as well as the proportions used to obtain baths having melting points adapted for use at the desired temperature of operation, will 30 be known to those experienced in the preparation and use of fused salt baths for heat treating metals and need not be discussed here.

Specific examples of preferred fused salt baths for practicing my invention are: 35

## Bath No. 1

Sodium cyanide: 15-30% by weight  
Remainder, sodium carbonate.

## Bath No. 2

Sodium cyanide, 2-20% by weight  
Remainder, equal parts of sodium carbonate  
and potassium carbonate.

## Bath No. 3

Sodium cyanide: 2-20% by weight  
Remainder, the mixture:

|                    | Per cent by weight |
|--------------------|--------------------|
| Barium chloride    | 50                 |
| Potassium chloride | 30                 |
| Sodium chloride    | 20                 |

## Bath No. 4

Same as Bath No. 3, but 0.05 to 0.5% by weight 55 of solid hydrocyanic acid polymer in place of the sodium cyanide.

In practicing my invention employing baths of compositions illustrated above various gaseous atmospheres may be employed to cover the fused 60

bath during operation. If an entirely inert or non-oxidizing atmosphere is employed, the bath will be substantially neutral, i. e., it will exert no substantial carburizing or decarburizing activity.

5 Illustrations of non-oxidizing gases which may be employed to render the bath inert are hydrogen, nitrogen, gaseous hydrocarbons; the rare gases such as argon, krypton, and helium; and ammonia. When it is desired that the bath have 10 a definite carburizing action, a suitable amount of an oxidizing substance is added to such an inert atmosphere. When there is present in the gaseous atmosphere over the bath a relatively small amount of an oxidizing constituent, a 15 definite but small carburizing activity will be exerted by the bath; the carburizing activity of the bath may be increased by increasing the amount of the oxidizing material present in the gaseous atmosphere.

20 I prefer to employ oxygen as the oxidizing material which is added to the gaseous atmosphere above the fused salt bath. However, other oxidizing substances may be employed in accordance with my invention in place of oxygen. For 25 the purpose of the present invention, gases such as carbon dioxide and water vapor are to be considered as oxidizing gases since their action upon the activity of a salt bath when they are added to the atmosphere above such a bath is, 30 generally speaking, the same as that produced when oxygen is added.

Care should be exercised in choosing the gases to be used in making up the gaseous atmosphere having a predetermined amount of an oxidizing constituent. Thus, mixtures of oxygen with hydrogen, carbon monoxide or ammonia should be avoided because of the explosive hazards involved. I prefer to employ mixtures of nitrogen with suitable amounts of oxygen as gaseous coverings for the fused salt baths when operated 40 in accordance with the present invention.

Methods for maintaining an atmosphere having a predetermined oxidizing value over the case hardening bath will be obvious to those 45 who are familiar with the art of heat treating metals and need not be described in detail here. It will be sufficient to state that the carburizing bath may be provided with a hood or muffle which is filled with the gaseous atmosphere containing the desired amount of an oxidizing substance. A convenient way of maintaining an atmosphere of suitable composition in the muffle is to pass continuously a mixture containing suitable proportions of an inert gas and an oxidizing gas into the aperture of the muffle through which the articles to be treated are inserted or removed from the bath. The gas mixture should be passed into the hooded space at such a rate that it streams out of the aperture (or 50 similar openings in the muffle) through which work pieces are inserted or removed, thereby preventing entrance into the hooded space of amounts of air such as would be sufficient to change substantially the composition of the gaseous atmosphere over the bath. If desired, suitable devices may be employed for passing the metal work into and out of the fused salt bath 55

so that the treatment may be carried out in a continuous manner. Thus when the case hardening of steel strip is involved, the steel strip may be passed continuously through a fused salt bath, by methods which are well known in the 5 art, so as to insure that a given portion of the strip remains immersed in the bath the required length of time to effect the desired case hardening. During operation, the carburizing activity of the bath is controlled as desired by maintaining over the bath a gaseous atmosphere containing a predetermined suitable proportion of oxygen or other suitable oxidizing gas.

In general, my invention may be practiced to effectively control the case hardening activity of 15 case hardening baths in which cyanide or other cyanogen compound is used as the case hardening ingredient. By varying the proportion of oxidizing gas in the atmosphere above the case hardening bath, the case hardening activity of the 20 bath may be varied accordingly. For example, a cyanide case hardening bath may be operated under an atmosphere of nitrogen or other non-oxidizing gas and a suitable proportion of oxygen or other oxidizing gas may be mixed with the 25 nitrogen. To decrease the activity of the bath, the atmosphere above the bath may for example consist of a nitrogen-oxygen mixture containing an oxygen concentration below that of the air, e. g., 1-5% by volume of oxygen. To increase the 30 activity of the bath, the covering atmosphere may, for example, consist of air to which oxygen has been added. This method of control is generally applicable to case hardening baths containing cyanogen compounds and is not restricted 35 to baths activated with cyanide.

My invention is not restricted to any particular temperature of heat treatment, but is generally applicable to the various heat treating temperatures commonly utilized for fused salt 40 bath metal heat treating operations, e. g., 450-900° C.

I claim:

1. A method for controlling the activity of a fused case hardening bath which contains a 45 cyanogen compound comprising maintaining said bath under an atmosphere of a gas containing a predetermined amount of an oxidizing gas.

2. A method for controlling the activity of a 50 fused case hardening bath which contains an alkali metal cyanide comprising maintaining said bath under an atmosphere of a gas containing a predetermined amount of oxygen.

3. A method for controlling the activity of a 55 fused case hardening bath which contains an alkali metal cyanide comprising maintaining said bath under an atmosphere of a gas mixture composed of a non-oxidizing gas and less than 20% by volume of oxygen.

4. A method for controlling the activity of a 60 fused case hardening bath which contains an alkali metal cyanide comprising maintaining said bath under an atmosphere of a gas mixture composed of a non-oxidizing gas and 1-5% by volume of oxygen.

DONALD A. HOLT.